# EUROPEAN PATENT SPECIFICATION

(11) **EP 1 511 572 B1**
(45) Date of publication and mention of the grant of the patent: **02.09.2009**
(21) Application number: 03728201.9
(22) Date of filing: 22.05.2003
(51) Int. Cl.: B02C 1/10, B02C 2/00, B02C 4/30, B02C 13/28

(54) **A WEAR PART INTENDED FOR A CRUSHER AND A METHOD OF MANUFACTURING THE SAME**
FÜR EINEN BRECHER BESTIMMTES VERSCHLEISSTEIL UND HERSTELLUNGSVERFAHREN DAFÜR
PIECE D'USURE POUR CONCASSEUR ET SON PROCEDE DE PRODUCTION

(30) Priority: 23.05.2002 SE 0201540
(43) Date of publication of application: 09.03.2005
(73) Proprietor: Sandvik Intellectual Property AB, 811 81 Sandviken (SE)
(72) Inventor: OLSSON ARTBERGER, Per, S-233 34 Svedala (SE); NILSSON, Anders, S-216 45 Malmö (SE); LANDEN, Pierre, S-241 35 Eslöv (SE)
(86) International application number: PCT/SE2003/000829
(87) International publication number: WO 2003/099443

(56) References cited:
- EP-A1- 0 785 289
- US-A- 5 340 530
- US-A- 6 086 003

## Description

### Field of the Invention

The present invention relates to a gyratory crusher or a jaw crusher wear part adapted to be detachable mounted on a supporting part of an impact-type multi-action crusher, the crusher being a gyratory crusher or a jaw crusher. The invention also relates to a method of manufacturing such a wear part.

### Background Art

Impact-type multi-action crushers, such as gyratory crushers and jaw crushers, crush a raw material, such as a stone block, ore block, concrete or brick block or the like, by a wear part being repeatedly moved towards the raw material to crush it against a counterbody. The wear part is supported by a supporting part which transmits the necessary force from a motor, moment arm, shaft or the like to the wear part. The crushing operation causes wear on the wear part, which therefore now and then must be detached from the supporting part and replaced.

For maximum life, the wear part is made of a material which has maximum abrasive resistance. The wear part is usually cast from what is referred to as Hadfield steels. These steels, which are described, for instance, in US 5,069,871 and EP 0 692 548, are austenitic manganese steels. A Hadfield steel has the property that the surface of the steel is hardened (deformation hardening) when the steel is acted upon by the raw material in the crusher, which results in good abrasive resistance.

For the supporting part to give sufficient support to the wear part, which is necessary to prevent the wear part from being deformed or cracking or from deforming the supporting part, the abutment surface of the wear part on the supporting surface of the supporting part must be machined to narrow tolerances. The problem is that the Hadfield steels also in such machining will be deformation-hardened, which makes machining difficult and time consuming.

### Summary of the Invention

The object of the present invention is to provide a wear part for an impact-type multi-action crusher, said wear part having good abrasive resistance and being easy to machine to narrow tolerances.

This object is achieved by a gyratory crusher or a jaw crusher wear part as claimed in claim 1.
By the wear part being divided into a body and a crushing layer, each part can be given the properties that are the most important ones for the part in question. Thus, the crushing layer is optimised for good abrasive resistance and the body for good machinability. By hot isostatic pressing, parts with complicated geometric structures can be produced also of materials that could otherwise not be used.

According to a preferred embodiment, the crushing layer is made of at least one powder material which has been subjected to hot isostatic pressing, the substance of which the body is made also having good weldability. There are a plurality of powder materials which are suitable as crushing layer and which can be subjected to hot isostatic pressing to form such a layer. A body which has good weldability is advantageous since the wear part is often fixed by welding.

Preferably, the crushing layer comprises at least two powder materials, which, without first being completely mixed with each other, have been subjected to hot isostatic pressing and which, after said pressing and subsequent aftertreatment, have different abrasive resistances, the crushing layer having portions of different abrasive resistances. The use of at least two materials makes it possible to vary the abrasive resistance of the crushing layer to obtain specific properties, such as improved abrasive resistance in some portions and lower abrasive resistance in other portions. Since the two materials are not mixed with each other, or at least not completely mixed with each other, there will, after the hot isostatic pressing, be portions with different abrasive resistances. If a highly abrasive resistant material, which is expensive, is used, this can be located in the portions of the crushing layer where the highest abrasive resistance is required, while a less expensive material can be used in the remaining portions. The material which after pressing and aftertreatment has the highest abrasive resistance is therefore conveniently arranged in the portions of the crushing layer where the greatest wear is to be expected. In this way, a more even wear is obtained over the surface of the wear part, which ensures a longer life of the wear part.

Preferably, the crushing layer and the body are joined by a bonding zone. The bonding zone, which may be formed, for instance, when a powder material in contact with a compact material is subjected to hot isostatic pressing, results in a safe connection between the body and crushing layer over the entire contact surface and renders it possible to do without a screw joint, weld joint and the like.

The body is suitably at least partly made of a substance selected from a group consisting of carbon steels and low alloy steels. These substances are easy to machine, have good weldability and are available at a low price. A body made of one of these substances can, for instance, be cast, machined or forged to the desired basic shape and then be finished to narrow tolerances. The body can also be made of a powder of one of the above substances, which is then subjected to hot isostatic pressing.

Preferably, a first portion of the crushing layer is made of at least one first powder material and, located downstream of said first portion in the direction of flow of the raw material, a second portion of the crushing layer is made of at least one second powder material, which, after subjecting the materials to hot isostatic pressing and subsequent aftertreatment, has higher abrasive resistance than the first material, whereby the second portion has higher abrasive resistance than the first portion. Wear is usually greatest in the portions located downstream in the direction of flow of the raw material since a larger number of objects are to be crushed in these portions. By locating the material having the highest abrasive resistance in these portions, it is thus possible to extend the life of the wear part. According to a still more preferred embodiment, the first material gradually merges into the second material in such a manner that the crushing layer obtains an abrasive resistance which increases gradually in the direction of flow of the raw material and which corresponds to the wear load in operation so that the profile of the wearing layer is kept essentially intact during the life of the wear part. This has the advantage that the crusher will have essentially the same and, thus, predictable capacity during the entire life of the wear part.

According to a preferred embodiment, the crushing layer has at least one protrusion protruding from the crushing layer and being made of at least one powder material which, after subjecting the powder materials to hot isostatic pressing and subsequent aftertreatment, has higher abrasive resistance than the powder material or materials of which the parts of the crushing layer which surround the protrusion are made. The protrusion will be exposed to particularly great wear load. At the same time the protrusion is, in the cases when it is being used, critical to the function of the wear part. By locating the most wear resistant material in the protrusion, the life of the wear part can thus be extended significantly.

According to another preferred embodiment, the crushing layer has at least one protrusion protruding from the crushing layer and being made by casting, sintering or forging and having higher abrasive resistance than the powder material or materials of which the parts of the crushing layer which surround the protrusion are made. Thus the protrusion can be made of materials, such as sintered tungsten carbide, which have excellent abrasion resistance but are better suited for other manufacturing methods than hot isostatic pressing. The protrusion can also be made of cast materials, such as Hadfield steels. Then it is possible to deformation-harden the protrusion in advance, before attaching it to the crushing layer. The parts of the crushing layer which surround and fix the protrusion are also in these cases made of at least one powder material which has been subjected to hot isostatic pressing.

The wear part can be an inner shell or an outer shell for use in a gyratory crusher. In gyratory crushers, the requirements for narrow tolerances in the abutment of the wear part on the supporting surface are strict, which makes the invention particularly suitable for this type of crushers.

According to a particularly preferred embodiment, the protrusion has the form of a rotationally symmetric step extending round the crushing layer. The step improves the crushing of the raw material and improves the grain shape of the crushed raw material.

According to a preferred embodiment, the crushing layer comprises at least two powder materials, which, after subjecting the materials to hot isostatic pressing, have different hardnesses, the softer of the two materials being located in a first layer closest to the body and the harder of the two materials being located in a second layer on the outside of the first layer. As a result, a very hard, but brittle, material can be used in the outer layer of the crushing layer and be supported by a softer material placed under the outer layer.

The object of the present invention is also to provide a method of manufacturing a wear part for an impact-type multi-action crusher, said wear part having great abrasive resistance and being easy to machine to narrow tolerances.

According to the invention, this object is achieved by a method as claimed in claim 14. By the wear part being divided into a body and a crushing layer, each part can be given the properties that are the most important ones for the part in question. Thus, the crushing layer is optimised for good abrasive resistance and the body for good machinability. By hot isostatic pressing, parts with complicated geometric structures can be manufactured. The abrasive resistant materials that are normally of interest for use in the crushing layer are often very difficult to machine to complicated geometric structures.

According to a preferred method, at least two powder materials, which after hot isostatic pressing and subsequent aftertreatment have different abrasive resistances, are introduced into the capsule without being completely mixed with each other, in such a manner that the material of the highest abrasive resistance is arranged in the parts of the capsule which correspond to the portions of the crushing layer where the greatest wear is to be expected. If a highly abrasive resistant material, which is expensive, is used, this can be located in the portions of the crushing layer where the highest abrasive resistance is required, while a less expensive material can be used in the remaining portions. A further advantage is that the wear on the wear part will be more even than if the same material is used in the entire crushing layer. Unevenly worn crushing layers constitute a common source of functional troubles and shortened life of wear parts.

Preferably, the body of the wear part is used as a wall in the capsule to be joined with the crushing layer. This saves a wall in the capsule that is used. Moreover, the advantage is achieved that the body and crushing layer are joined by a bonding zone which will be very strong since it covers the entire surface where the body and the crushing layer are in contact with each other. Nor is a weld joint, bolt joint or the like required to hold the body and the crushing layer together.

According to a preferred method, at least one first powder material is introduced into a first part of the capsule which corresponds to a first portion of the crushing layer and at least one second powder material is introduced into a second part of the capsule which corresponds to a second portion of the crushing layer, which second portion is located downstream of the first portion in the direction of flow of the raw material, the second material in the second portion, after subjecting the materials to hot isostatic pressing and subsequent aftertreatment, having higher abrasive resistance than the first material. Uneven wear is a great problem in many crushers, especially in gyratory crushers. Owing to the wear which usually is greatest in the portions positioned downstream in the direction of flow of the raw material, the crusher capacity of crushing a raw material is reduced and, after a certain period of operation of the wear part, the crusher cannot crush the raw material to the same small sizes, and therefore the wear part must be replaced. By a more abrasive resistant material being used in the portion of the crushing layer which is close to the end point of the flow of raw material, the life of the wear part can be increased significantly. According to a particularly preferred method, the first material and the second material are introduced into the capsule in such a manner that the first material gradually merges into the second material, the crushing layer obtaining an abrasive resistance that increases gradually in the direction of flow of the raw material and corresponds to the wear load in operation, so that the profile of the crushing layer is kept essentially intact during the life of the wear part. As mentioned above, this has the advantage that the performance of the crusher will be constant and thus predictable for the entire life of the crusher.

According to a preferred method, the crushing layer is manufactured with at least one protrusion protruding from the crushing layer, at least one powder material being introduced into the capsule in the parts of the capsule which correspond to the protrusion and at least one other powder material being introduced into the parts of the capsule which correspond to the parts of the crushing layer which surround the protrusion, the material of the protrusion, after subjecting the materials to hot isostatic pressing and subsequent aftertreatment, having higher abrasive resistance than the material of the parts of the crushing layer which surround the protrusion. As mentioned above, the life of the protrusion will thus be increased, which ensures the above advantages of longer life for the entire wear part.

According to another preferred method, the protrusion is manufactured in a first step by hot isostatic pressing, after which the parts of the crushing layer which surround the protrusion are manufactured in a second step. This method results in improved control of the conditions under which the protrusion is manufactured. The extent and connection surfaces of the protrusion to the surrounding material can also be formed with greater accuracy. It is also possible to make the protrusion of a material that requires hot isostatic pressing in conditions, as regards, for instance, temperature and pressure, that are unsuitable for the surrounding material.

According to another preferred method, the crushing layer has at least one protrusion protruding from the crushing layer and being made in a first step by sintering, casting or forging, the protrusion in a second step being arranged in the capsule and at least one powder material being introduced into the parts of the capsule which correspond to the parts of the crushing layer which surround the protrusion, the protrusion, after subjecting the materials to hot isostatic pressing and subsequent aftertreatment, having higher abrasive resistance than the parts of the crushing layer which surround the protrusion. As mentioned above, this makes it possible to select for the protrusion also such abrasive resistant materials as are not best suited for hot isostatic pressing.

According to a preferred method, the protrusion is formed as a step. The step ensures, as mentioned above, advantages in crushing.

Preferably, the body is at least partly made of a substance selected from a group consisting of carbon steels and low alloy steels. Owing to these substances, the abutment surface of the body is easy to machine to narrow tolerances, as mentioned above.

### Brief Description of the Drawings

The invention will now be described in more detail by way of embodiments and with reference to the accompanying drawings.
Fig. 1 shows a gyratory crusher.
Fig. 2 is a cross-sectional view of a portion of the crusher in Fig. 1 and shows an inner shell and an outer shell according to prior art.
Fig. 3 is a cross-sectional view and shows a wear part according to the invention in a first embodiment, formed as an inner shell.
Fig. 4 is a cross-sectional view and shows a wear part according to the invention in a second embodiment, formed as an inner shell.
Fig. 5 is a cross-sectional view and shows a wear part of the invention in a third embodiment, formed as an inner shell.
Fig. 6 is a cross-sectional view and shows a wear part according to the invention in a fourth embodiment, formed as an inner shell.
Fig. 7 is a cross-sectional view and shows wear parts according to the invention formed as an inner shell and an outer shell, intended for a crusher that is normally used in coarse crushing.
Fig. 8 is a cross-sectional view and shows a capsule for manufacturing wear parts according to the invention.

### Description of Preferred Embodiments

Fig. 1 shows a gyratory crusher 1. The crusher 1 has a crusher shaft 2 which at its lower end 3 is eccentrically mounted. In its upper portion, the crusher shaft 2 has a crushing head 4. The crushing head 4 has an inner shell 5, which in the simultaneous rotary and oscillating motions of the crusher shaft 2 crushes raw materials, that are supplied to the upper portion 6 of the crusher 1, against an outer shell 7. A crushing chamber 8 is formed between the inner shell 5 and the outer shell 7. As a rule, the function of the crusher 1 is determined by the gap S which is the smallest distance between the inner shell 5 and the outer shell 7 of the crusher 1. The crusher shaft 2 can by means of an adjusting device 9 be moved in the vertical direction. Thus, the gap S of the crushing chamber 8 can be adjusted, thus allowing setting in a desirable manner the relation between the amount of material that is crushed by the crusher 1 and the size of the crushed material.

Fig. 2 shows an inner shell 5' and an outer shell 7' of prior-art type. As illustrated, the inner shell 5' is supported by a supporting part in the form of a support cone 10 included in the crushing head 4 and the outer shell 7' on a supporting part 11 in the form of an intermediate ring. The inner shell 5' is held on the support cone 10 by a nut 12, which by means of a ring 13, that is welded to the inner shell 5' and the nut 12, holds the inner shell 5' on the support cone 10. The outer shell 7' is attached to a base 11' by means of a bolt joint. When operating the crusher, raw materials are supplied to the inlet 14 of the crusher and conveyed in the direction of flow P of the raw material, (in Fig. 2 indicated by an arrow) downwards through the crusher 1. According to prior-art technique, both the inner shell 5' and the outer shell 7' are made of cast manganese steel. The abutment surface 15 of the inner shell 5' on the support cone 10 is machined to narrow tolerances in complicated turning operations. In the same way, the abutment surfaces 16 of the outer shell 7' on the supporting part 11 are machined to narrow tolerances. To ensure a correct gap S, usually also the crushing surface 17 of the inner shell 5' and the crushing surface 18 of the outer shell 7' are machined by means of complicated turning operations.

The dashed lines in Fig. 2 indicate the extent of the inner shell 5' and the outer shell 7' after a period of wear. The wear makes it necessary to move the crusher shaft 2 upwards to maintain a constant gap S. When the crusher shaft 2 has reached its uppermost position, the inner shell 5' must be replaced without its upper portion being worn out.

Fig. 3 shows a first embodiment of a wear part according to the invention in the form of an inner shell 5 for the gyratory crusher 1. The inner shell 5 has a body 19 made of a carbon steel which is easy to machine. The abutment surface 15 of the body 19 for abutment on the support cone 10 has been turned to narrow tolerances for a good fit to the support cone 10. The inner shell 5 has a crushing layer 20. The crushing layer 20 is made of two different powder materials 21 and 22, for instance Elmax and Vanadis 10 made by Uddeholm AB, SE, which have been subjected to hot isostatic pressing.

In hot isostatic pressing the body 19 and the crushing layer 20 will be partly joined by diffusion and form a bonding zone 20' which extends along the entire contact surface between the body 19 and the crushing layer 20.

In the embodiment shown in Fig. 3, two powder materials 21, 22 are used in the crushing layer 20 as mentioned above. The first material 21 is placed at the end, located at the inlet 14, of the inner shell 5 in a first portion 21' of the crushing layer 20, and the second material 22 is placed in a second portion 22' of the crushing layer 20, which is positioned downstream of the first portion 21' in the direction of flow P of the raw material. The materials 21, 22 are selected so that the second material 22 has higher abrasive resistance than the first material 21 after both materials being subjected to hot isostatic pressing. In a portion 23 of the crushing layer 20, the first material 21 gradually merges into the second material 22 in the direction of flow P of the raw material. In the embodiment in Fig. 3, uneven wear that arises in prior-art technique (Fig. 2) is thus avoided owing to the fact that the abrasive resistance of the crushing layer 20 along the direction of flow P of the raw material has been adjusted to the actual wear. As is evident from Fig. 3, the crushing layer 20 has on its outside a special curvature. This curvature, which is described, for instance, in GB 2,123,314, is intended to maintain a constant inlet 14 as the crusher shaft 2 moves upwards subsequent to wear. Thus the inner shell 5 will have an almost constant profile during its entire life, which ensures that the correct gap S can be set without the capacity of the crusher 1 decreasing.

Fig. 4 shows a second embodiment of a wear part according to the invention in the form of an inner shell 5. Like in the embodiment shown in Fig. 3, this inner shell 5 has a body 19 having an abutment surface 15 and being made in the manner as described above, and a crushing layer 20. The crushing layer 20 has, in its portion positioned at the inlet 14, a number of shoulders or steps 24, 25. The steps 24, 25, which can be resembled to rotationally symmetric stairs extending round the crushing layer 20 and which are positioned upstream of a portion 26, improve the possibility of crushing the raw material to smaller pieces and also improve the grain shape of the crushed raw material. The steps 24, 25, which in operation are exposed to heavy wear, are made of a powder material 27 having a higher abrasive resistance than the material 28 of which the remainder of the crushing layer 20 is made, after the materials being exposed to hot isostatic pressing. The steps 24, 25 will thus last longer than in the case if they had also been made of the material 28, thereby increasing the operating time in which the shell 5 exhibits the desired function.

The steps 24, 25 can be made at the same time as the remainder of the crushing layer 20 in the above isostatic pressing. However, it is also possible to make the steps 24, 25 in a first step, i.e. a first processing step, by hot isostatic pressing and then in a second step, i.e. a second processing step, make the remainder of the crushing layer. It is also possible to make the steps 24, 25 by casting, sintering, for instance of tungsten carbide, or forging, after which the parts of the crushing layer 20 which surround the steps 24, 25 are made of a powder material that is subjected to hot isostatic pressing.

Fig. 5 illustrates a third embodiment of a wear part according to the invention in the form of an inner shell 5. This embodiment differs from the embodiment shown in Fig. 4 essentially only by its inner shell 5 having larger shoulders or steps 29. The steps 29, which may be resembled to rotationally symmetric stairs extending round the crushing layer 20, give the advantage that a smaller crushing surface 30 is obtained, thus allowing the raw material to be crushed with greater force against this surface 30. The steps 29 thus prevent large objects from reaching the crushing surface 30. A certain degree of wear by the raw material also takes place in the area of the steps 29.

Fig. 6 illustrates a fourth embodiment of a wear part according to the invention in the form of an inner shell 5. In this embodiment, the crushing layer 20 has at least two different layers 31, 32, viz. a lower layer 31 closest to the body 19 and an upper layer 32 which is harder than the lower layer 31. The hard, but brittle, layer 32 is supported by the softer lower layer 31. The outer surface of the harder layer 32 thus constitutes the crushing surface 17 of the crushing layer 20.

Both the softer layer 31 and the harder layer 32 are made by hot isostatic pressing of powder materials. The layers 31, 32 can be made simultaneously. Alternatively, the softer layer 31 can be made in a first step and the harder layer 32 can be made in a subsequent second step. It is also possible to make the lower layer 31 of a cast manganese steel, for instance a Hadfield steel. The manganese steel has relatively high abrasive resistance, which is advantageous if the upper layer 32 should be damaged at any point.

Fig. 7 illustrates a primary gyratory crusher 33.
The primary gyratory crusher 33 is a type of gyratory crusher which is used for crushing large objects. Thus, the inlet 14 is very wide. The outer shell 34 of the primary gyratory crusher 33 is divided into a number of segments 35, 36 which are attached to a supporting part 11. The segment 35 has a crushing layer 37 which is made of a powder material that has been subjected to hot isostatic pressing and that is attached to a body 38. The body 38 is made of a carbon steel. The segment 36 positioned downstream of the segment 35 in the direction of flow P of the raw material has a crushing layer 39 which is made by hot isostatic pressing and is attached to a body 38. The crushing layer 39 has higher abrasive resistance than the crushing layer 37. Since the wear is smaller in the portions of the crusher 33 which are positioned close to the inlet 14, the segments 35, 36 will be worn at approximately the same rate in operation of the crusher, which ensures an even profile of the outer shell 34. The crusher 33 also has an inner shell 5 which is replaceably attached to a support cone 10. This shell 5 can be formed in the manner as described above with reference to Figs 3-6.

The hot isostatic pressing, which is described, for instance, in US 3,695,597, is carried out by means of a capsule 40 (see Fig. 8). In the capsule 40, the body 19 is used as a wall. Otherwise, the capsule 40 has the geometric shape that is desired for the completed inner shell 5. Steps 29, if any, that have been made in advance by, for instance, hot isostatic pressing, sintering, casting or forging, are placed in the capsule 40 in the positions as required in the completed crushing layer 20. In the capsule 40, at least one powder material is introduced in at least one opening 41. After vibrating, degassing and sealing, the capsule 40 is exposed to heat and pressure, whereby the powder material is deformed and joined by diffusion. The capsule 40 can then be removed. In some cases, the capsule 40 is joined with the crushing layer 20 and becomes part thereof. After subsequent treatment, comprising, for instance, tempering, the inner shell 5 is ready for use. Owing to the conditions in pressing, the crushing surface 17 of the shell 5 need not be machined at all but satisfies the tolerances that are required for the selected gap S. The abutment surface 15 of the body 19 can be machined either before pressing or after the same.

It will appreciated that a number of modifications of the embodiments described above are feasible within the scope of the invention.

Thus, for instance an inner shell 5 or an outer shell 7 can be formed, in which the steps 24, 25, 29 shown in Figs 4 and 5 are combined with a crushing layer 20 containing the combinations of powder materials 21, 22, 31, 32 shown in Fig. 3 and/or Fig. 6, said materials being subjected to hot isostatic pressing with a view to forming different portions and layers. Of course, a plurality of, for instance 2-7, different powder materials can be used for the different layers, portions and steps of the wear part. The materials can either merge more or less gradually into each other or be separated by distinct limits. Such limits may consist of, for instance, thin metal foils that are inserted into the capsule 40.

Wear parts according to the invention can be manufactured, inter alia, for the above-described gyratory crushers and jaw crushers. Jaw crushers in general are described, for instance, in WO 00/25926 and US 4,927,089. A jaw crusher has two jaws each having the shape of a relatively flat surface, one jaw crushing the raw material against the other jaw by a reciprocating motion. A raw material is introduced into the upper portion of the jaw crusher and passed downwards through the crusher in an essentially vertically downward direction of flow of the raw material. When passing downwards through the jaw crusher, the raw material will be crushed a plurality of times to increasingly smaller dimensions. The jaws comprise supporting parts to which wear parts according to the invention can be attached by welding or bolting. A great deal of the wear will arise in the lower parts of the jaw crusher where a very large number of objects of the raw material are to be crushed. In many cases it will thus be convenient to use wear parts in the jaw crusher that have been manufactured, for instance, according to the principles as described in connection with Figs 3 and 7. Gyratory crushers and jaw crushers are impact-type multi-action crushers, i.e. crushers in which a piece of the raw material is crushed several times while passing through the crusher and by impact between two surfaces that are accelerated towards each other and strike against the raw material.

The body 19 is made of a substance which is easy to machine but which at the same time has the mechanical strength that is necessary to support the crushing layer 20. The body can be cast, forged or cold- and/or hot-worked to the correct shape. Since the body is not in contact with the raw material, it can be made of a substance of low abrasive resistance. Low abrasive resistance often makes the substance easy to machine. The substances that are most convenient for the body are carbon steels and low alloy steels. The abutment surface 15, 16 of the body on the supporting part 10, 11 can be machined to narrow tolerances, for instance by turning, milling or grinding.

Substances that are easy to weld are particularly advantageous as substance for the body. The wear part can be attached to the supporting part by means of a weld that should resist high loads. Particularly suitable substances are therefore carbon steels and lower alloy steels.

The segments 35, 36 illustrated in Fig. 7 can also each be formed according to the principles described above in connection with Figs 3-6. Thus, wear parts for gyratory crushers as well as jaw crushers can be made in several segments. Each segment may either comprise a single powder material or a plurality of materials. The segments may also comprise steps.

When a plurality of steps 24, 25, 29 are used, they can be made of the same material, but also of different materials and by different methods. For instance, it is possible to make the steps 24 of a powder material that is subjected to hot isostatic pressing, and the step 25 of a still harder material which has been made in advance by sintering.

It is also possible to manufacture a body and a crushing layer each separately, for instance by casting, machining, forging or hot isostatic pressing, and then attach the body and the crushing layer to each other by hot isostatic pressing, also referred to as diffusion bonding.

## Claims

1. A gyratory crusher or a jaw crusher wear part adapted to be detachable mounted on a supporting part (10, 11) of an impact-type multi-action crusher (1), the crusher (1) being a gyratory crusher or a jaw crusher, **characterised in that** the wear part (5, 7, 34) is at least partly manufactured by hot isostatic pressing and that the wear part (5, 7, 34) has a body (19, 38) adapted to mount the wear part (5, 7, 34) on the supporting part (10, 11) and a crushing layer (20, 37, 39) which is attached to the body (19, 38) and adapted to be brought, during operation of the crusher (1), into repeated contact with a raw material which is to be crushed, the body (19, 38) being made of a substance which is easy to machine to narrow tolerances, and the crushing layer (20, 37, 39) being made of a material (21, 22, 27, 28) of high abrasive resistance.

2. A wear part as claimed in claim 1, in which the crushing layer (20, 37, 39) is made of at least one powder material (21, 22, 27, 28) which has been subjected to hot isostatic pressing, and in which the substance of which the body (19, 38) is made has also good weldability.

3. A wear part as claimed in claim 1 or 2, in which the crushing layer (20, 37, 39) comprises at least two powder materials (21, 22, 27, 28), which, without first being completely mixed with each other, have been subjected to hot isostatic pressing and which materials (21, 22, 27, 28), after said pressing and subsequent aftertreatment, have different abrasive resistances, the crushing layer (20, 37, 39) having portions (21', 22' 23, 24, 25, 26, 29) of different abrasive resistances.

4. A wear part as claimed in claim 3, in which the powder material (22, 27) which after pressing and subsequent aftertreatment has the highest abrasive resistance is arranged in the portions (22', 24, 25, 29) of the crushing layer (20, 37, 39) where the greatest wear is to be expected.

5. A wear part as claimed in any one of the preceding claims, in which the crushing layer (20, 37, 39) and the body (19, 38) are joined by a bonding zone (20').

6. A wear part as claimed in any one of the preceding claims, in which the body (19, 38) is at least partly made of a substance selected from a group consisting of carbon steels and low alloy steels.

7. A wear part as claimed in any one of the preceding claims, in which a first portion (21') of the crushing layer (20) is made of at least one first powder material (21) and, located downstream of said first portion (21') in the direction of flow (P) of the raw material, a second portion (22') of the crushing layer (20) is made of at least one second powder material (22), which, after the materials (21, 22) being subjected to hot isostatic pressing and subsequent aftertreatment, has higher abrasive resistance than the first material (21), the second portion (22') having higher abrasive resistance than the first portion (21').

8. A wear part as claimed in claim 7, in which the first material (21) gradually merges into the second material (22) in such a manner that the crushing layer (20) obtains an abrasive resistance which increases gradually in the direction of flow of the raw material (P) and which corresponds to the wear load in operation so that the profile of the crushing layer (20) is kept essentially intact during the life of the wear part (5, 7).

9. A wear part as claimed in any one of claims 3, 4, 7 and 8, in which the crushing layer (20) has at least one protrusion (24, 25, 29) protruding from the crushing layer (20) and being made of at least one powder material (27) which, after subjecting the powder materials (27, 28) to hot isostatic pressing and subsequent aftertreatment, has higher abrasive resistance than the powder material or materials (28) of which the parts of the crushing layer (20) which surround the protrusion (24, 25, 29) are made.

10. A wear part as claimed in any one of claims 3, 4, 7 and 8, in which the crushing layer (20) has at least one protrusion (24, 25, 29) protruding from the crushing layer (20) and being made by casting, sintering or forging and having higher abrasive resistance than the powder material or materials (28) of which the parts of the crushing layer (20) which surround the protrusion (24, 25, 29) are made.

11. A wear part as claimed in any one of the preceding claims, which is an inner shell (5) or an outer shell (7) for use in a gyratory crusher (1),

12. A wear part as claimed in claim 11 and any one of claims 9 and 10, in which the protrusion has the form of a rotationally symmetric step (24, 25, 29) extending round the crushing layer (20).

13. A wear part as claimed in any one of the preceding claims, in which the crushing layer (20) comprises at least two powder materials, which, after subjecting the materials to hot isostatic pressing, have different hardnesses, the softer of the two materials being located in a first layer (31) closest to the body (19) and the harder of the two materials being located in a second layer (32) on the outside of the first layer (31).

14. A method of manufacturing a wear part for detachable mounting on a supporting part (10, 11) in an impact-type multi-action crusher (1), the crusher (1) being a gyratory crusher or a jaw crusher, **characterised in that** the wear part (5, 7, 34) is manufactured as a body (19, 38) for mounting of the wear part (5, 7, 34) on the supporting part (10, 11) and a crushing layer (20, 37, 39) which is attached to the body (19, 38) and adapted to be brought, during operation of the crusher (1), into repeated contact with a raw material which is to be crushed, the body (19, 38) being made of a substance which is easy to machine to narrow tolerances, and the crushing layer (20, 37, 39) being made of a material (21, 22, 27, 28) of high abrasive resistance by at least one powder material (21, 22, 27, 28) being introduced into a capsule (40), the capsule (40) being degassed and sealed and the material (21, 22, 27, 28) in the capsule (40) being subjected to hot isostatic pressing, after which the wear part (5, 7, 34) is subjected to aftertreatment.

15. A method as claimed in claim 14, in which at least two powder materials (21, 22, 27, 28), which after hot isostatic pressing and subsequent aftertreatment have different abrasive resistances, are introduced into the capsule (40) without being completely mixed with each other, in such a manner that the material (22, 27) of the highest abrasive resistance is arranged in the parts of the capsule (40) which correspond to the portions (22', 24, 25, 29) of the crushing layer (20, 37, 39) where the greatest wear is to be expected.

16. A method as claimed in claim 14 or 15, in which the body (19, 38) of the wear part (5, 7, 34) is used as a wall in the capsule (40) to be joined with the crushing layer (20, 37, 39).

17. A method as claimed in any one of claims 14-16, in which at least one first powder material (21) is introduced into a first part of the capsule (40) which corresponds to a first portion (21') of the crushing layer (20) and at least one second powder material (22) is introduced into a second part of the capsule (40) which corresponds to a second portion (22') of the crushing layer (20), which is located downstream of the first portion (21') in the direction of flow of the raw material (P), the second material (22) in the second portion (22'), after subjecting the materials (21, 22) to hot isostatic pressing and subsequent aftertreatment, having higher abrasive resistance than the first material (21).

18. A method as claimed in claim 17, in which the first material (21) and the second material (22) are introduced into the capsule (40) in such a manner that the first material (21) gradually merges into the second material (22), the crushing layer (20) obtaining an abrasive resistance that increases gradually in the direction of flow of the raw material (P) and corresponds to the wear load in operation, so that the profile of the crushing layer (20) is kept essentially intact during the life of the wear part (5, 7).

19. A method as claimed in any one of claims 14-18, in which the crushing layer (20) is manufactured with at least one protrusion (24, 25, 29) protruding from the crushing layer (20), at least one powder material (27) being introduced into the capsule (40) in the parts of the capsule (40) which correspond to the protrusion (24, 25, 29) and at least one other powder material (28) being introduced into the parts of the capsule (40) which correspond to the parts of the crushing layer (20) which surround the protrusion (24, 25, 29), the material (27) of the protrusion (24, 25, 29), after subjecting the materials (27, 28) to hot isostatic pressing and subsequent aftertreatment, having higher abrasive resistance than the material (28) of the parts of the crushing layer (20) which surround the protrusion (24, 25, 29).

20. A method as claimed in claim 19, in which the protrusion (24, 25, 29) is manufactured in a first step by hot isostatic pressing, after which the parts of the crushing layer (20) which surround the protrusion (24, 25, 29) are manufactured in a second step.

21. A method as claimed in any one of claims 14-18, in which the crushing layer (20) has at least one protrusion (24, 25, 29) protruding from the crushing layer (20) and being made in a first step by sintering, casting or forging, the protrusion (24, 25, 29) in a second step being arranged in the capsule (40) and at least one powder material (28) being introduced into the parts of the capsule (40) which correspond to the parts of the crushing layer (20) which surround the protrusion (24, 25, 29), the protrusion (24, 25, 29), after subjecting the materials to hot isostatic pressing and subsequent aftertreatment, having higher abrasive resistance than the parts of the crushing layer (20) which surround the protrusion (24, 25, 29).

22. A method as claimed in any one of claims 19-21, in which the protrusion is formed as a step (24, 25, 29).

23. A method as claimed in any one of claims 14-22, in which the body (19, 38) is at least partly made of a substance selected from a group consisting of carbon steels and low alloy steels.

## Patentansprüche

1. Verschleißteil für einen Kreiselbrecher oder einen Backenbrecher, welches dafür ausgelegt ist, lösbar an einem Stützteil (10, 11) eines Schlagbrechers (1) mit Mehrtachanwendungen montiert zu werden, wobei der Brecher (1) ein Kreiselbecher oder ein Backenbrecher ist, **dadurch gekennzeichnet, daß** das Verschleißteil (5, 7, 34) wenigstens teilweise durch isostatisches Heißpressen hergestellt ist und daß das Verschleißteil (5, 7, 34) einen Hauptteil (19, 38), der dafür ausgelegt ist, das Verschleißteil (5, 7, 34) an dem Stützteil (10, 11) zu befestigen, und eine Blechschicht (20, 37, 39) aufweist, die an dem Hauptteil (19, 38) angebracht ist und dafür ausgelegt ist, während des Betriebs des Brechers (1) wiederholt mit einem zu brechenden Rohrmaterial in Kontakt zu treten, wobei der Hauptteil (19, 38) aus einer Substanz hergestellt ist, die leicht auf enge Toleranzen bearbeitet werden kann, und die Brechschicht (20, 37, 39) aus einem Material (21, 22, 27, 28) mit hoher Abrasionsbeständigkeit hergestellt ist.

2. Verschleißteil nach Anspruch 1, wobei die Brechschicht (20, 37, 39) aus wenigstens einem pulverförmigen Material (21, 22, 27, 28) hergestellt ist, welches isostatischem Heißpressen unterworfen wurde, und wobei die Substanz, aus welcher der Hauptteil (19, 38) hergestellt ist, auch eine gute Schweißbarkeit besitzt.

3. Verschleißteil nach einem der Ansprüche 1 oder 2, wobei die Brechschicht (20, 27, 39) wenigstens zwei pulverförmige Materialien (21, 22, 27, 28) aufweist, die, ohne zuerst vollständig miteinander gemischt zu werden, isostatischem Heißpressen unterworfen wurden und die nach dem Pressen und der anschließenden Nachbehandlung verschiedene Abrasionsbeständigkeiten haben, wobei die Brechschicht (20, 37, 39) Abschnitte (21', 22', 23, 24, 25, 26, 29) mit verschiedenen Abrasionsbeständigkeiten aufweist.

4. Verschleißteil nach Anspruch 3, wobei das pulverförmige Material (22, 27), welches nach dem Pressen und der anschließenden Nachbehandlung die höchste Abrasionsbeständigkeit besitzt, in den Abschnitten (22', 24, 25, 29) der Brechschicht (20, 37, 39) angeordnet ist, in welchen der größte Verschleiß zu erwarten ist.

5. Verschleißteil nach einem der vorangegangenen Ansprüche, wobei die Brechschicht (20, 37, 39) und der Hauptteil (19, 38) durch eine Bindungszone (20') miteinander verbunden sind.

6. Verschleißteil nach einem der vorangegangenen Ansprüche, wobei der Hauptteil (19, 38) zumindest teilweise aus einer Substanz hergestellt ist, die aus einer Gruppe ausgewählt ist, bestehend aus Kohlenstoffstählen und niedrig legierten Stählen.

7. Verschleißteil nach einem der vorangegangenen Ansprüche, wobei ein erster Abschnitt (21') der Brechschicht (20) aus wenigstens einem ersten pulverförmigen Material (21) hergestellt ist und stromabwärts von dem ersten Abschnitt (21') in Fließrichtung (P) des Rohmaterials ein zweiter Abschnitt (22') der Blechschicht (20) aus wenigstens einem zweiten pulverförmigen Material (22) hergestellt ist, welches, nachdem die Materialien (21, 22) isostatischem Heißpressen und anschließender Nachbehandlung unterworfen wurden, eine höhere Abrasionsbeständigkeit besitzt als das erste Material (21), wobei der zweite Abschnitt (22') eine höhere Abrasionsbeständigkeit besitzt als der erste Abschnitt (21').

8. Verschleißteil nach Anspruch 7, wobei sich das erste Material (21) auf eine solche Weise allmählich mit dem zweiten Material (22) vereinigt, daß die Brechschicht (20) eine Abrasionsbeständigkeit erhält, die in der Fließrichtung des Rohmaterials (P) allmählich zunimmt und der Verschleißlast im Betrieb entspricht, so daß das Profil der Brechschicht (20) während der Lebensdauer des Verschleißteils (5, 7) im wesentlichen intakt gehalten wird.

9. Verschteißteil nach einem der Ansprüche 3, 4, 7 und 8, wobei die Brechschicht (20) wenigstens einen Vorsprung (24, 25, 29) aufweist, der von der Brechschicht (20) vorspringt und aus wenigstens einem pulverförmigen Material (27) hergestellt ist, welches, nachdem die pulverförmigen Materialien (27, 28) isostatischem Heißpressen und anschließender Nachbehandlung unterworfen wurden, eine höhere Abrasionsbeständigkeit besitzt als das pulvorförmige Material oder die Materialien (28), aus welchem bzw. welchen die Teile der Brechschicht (20), welche den Vorsprung (24, 25, 29) umgeben, hergestellt sind.

10. Verschleißteil nach einem der Ansprüche 3, 4, 7 und 8, wobei die Brechschicht (20) wenigstens einen Vorsprung (24, 25, 29) aufweist, der von der Brechschicht (20) vorspringt und durch Gießen, Sintern oder Schmieden hergestellt ist und eine höhere Abrasionsbeständigkeit besitzt als das pulverförmige Material oder die Materialien (28), aus welchem bzw. welchen die Teile der Brechschicht (20), welche den Vorsprung (24, 25, 29) umgeben, hergestellt sind.

11. Verschleißteil nach einem der vorangegangenen Ansprüche, welches eine innere Mantelfläche (5) oder eine äußere Mantelfläche (7) zur Verwendung in einem Kreiselbrecher (1) ist.

12. Verschleißteil nach Anspruch 11 und irgendeinem der Ansprüche 9 und 10, wobei der Vorsprung die Form einer rotationssymmetrischen Stufe (24, 25, 29) hat, die sich um die Brechschicht (20) herum erstreckt.

13. Verschleißteil nach einem der vorangegangenen Ansprüche, wobei die Brechschicht (20) wenigstens zwei pulverförmige Materialien aufweist, welche, nachdem die Materialien isostatischem Heißpressen unterworfen wurden, verschiedene Härten haben, wobei sich das weichere der beiden Materialien in einer ersten Schicht (31) befindet, die dem Hauptteil (19) am nächsten liegt, und sich das härtere der beiden Materialien in einer zweiten Schicht (32) an der Außenseite der ersten Schicht (31) befindet

14. Verfahren zum Herstellen eines Verschleißteils für das lösbare Befestigen an einem Stützteil (10, 11) in einem Schlagbrecher (1) mit Mehrfachanwendungen, wobei der Brecher (1) ein Kreiselbrecher oder ein Backenbrecher ist, **dadurch gekennzeichnet, daß** das Verschleißteil (5, 7, 34) als ein Hauptteil (19, 38) für das Befestigen des Verschleißteils (5, 7, 34) an dem Stützteil (10, 11) und eine Brechschicht (20, 37, 39) hergestellt ist, die an dem Hauptteil (19, 38) angebracht und dafür ausgelegt ist, während des Betriebs des Brechers (1) in wiederholten Kontakt mit einem zu brechenden Rohmaterial zu treten, wobei der Hauptteil (19, 38) aus einer Substanz hergestellt ist, die leicht auf enge Toleranzen bearbeitet werden kann, und die Brechschicht (20, 37, 39) aus einem Material (21, 22, 27, 28) mit hoher Abraslonsbeständlgkelt hergestellt wird, indem wenigstens ein pulverförmiges Material (21, 22, 27, 28) in eine Kapsel (40) eingebracht wird, die Kapsel (40) entgast und versiegelt wird und das Material (21, 22, 27, 28) in der Kapsel (40) isostatlschem Heißpressen unterworfen wird, wonach das Verschleißteil (5, 7, 34) einer Nachbehandlung unterworfen wird.

15. Verfahren nach Anspruch 14, wobei wenigstens zwei pulverförmige Materialien (21, 22, 27, 28), die nach dem isostatischen Heißpressen und der anschließenden Nachbehandlung verschiedene Abrasionsbeständigkeiten haben, ohne vollständiges Vermischen miteinander auf eine solche Weise in die Kapsel (40) eingebracht werden, daß das Material (22, 27) mit der höchsten Abrasionabeständigkeit in den Teilen der Kapsel (40) angeordnet ist, welche den Abschnitten (22', 24, 25, 29) der Brechschicht (20, 37, 39) entsprechen, wo der größte Verschleiß zu erwarten ist.

16. Verfahren nach Anspruch 14 oder 15, wobei der Hauptteil (19, 38) des Verschleißteils (5, 7, 34) als eine Wand in der Kapsel (40) verwendet wird, um mit der Brechschicht (20, 37, 39) verbunden zu werden.

17. Verfahren nach einem der Ansprüche 14 bis 16, wobei wenigstens ein erstes pulverrormiges Material (21) in einen ersten Teil der Kapsel (40) eingebracht wird, welcher einem ersten Abschnitt (21') der Brechschicht (20) entspricht, und wenigstens ein zweites pulverförmiges Material (22) in einen zweiten Teil der Kapsel (40) eingebracht wird, welcher einem zweiten Abschnitt (22') der Blechschicht (20) entspricht, welcher in Fließrichtung des Rohmaterials (P) stromabwärts von dem ersten Abschnitt (21') liegt, wobei das zweite Material (22) in dem zweiten Abschnitt (22'), nachdem die Materialien (21, 22) lsostatischem Heißpressen und anschließender Nachbehandlung unterworfen wurden, eine höhere Abrasionsbeständigkelt aufweist als das erste Material (21).

18. Verfahren nach Anspruch 17, wobei das erste Material (21) und das zweite Material (22) auf eine solche Weise in die Kapsel (40) eingebracht werden, daß das erste Material (21) sich alimählich mit dem zweiten Material (22) vereinigt, wobei die Brechschicht (20) eine Abrasionsbeständigkeit erhält, die in der Fließrichtung des Rohmaterials (P) allmählich zunimmt und der Verschleißlast im Betrieb entspricht, so daß das Profil der Brechschicht (20) während der Lebensdauer des Verschleißteils (5, 7) im wesentlichen intakt gehalten wird.

19. Verfahren nach einem der Ansprüche 14 bis 18, wobei die Blechschicht (20) mit wenigstens einem Vorsprung (24, 25, 29) hergestellt wird, welcher von der Brechschicht (20) vorspringt, wobei wenigstens ein pulverförmiges Material (27) in die Kapsel (40) in diejenigen Teile der Kapsel (40), die dem Vorsprung (24, 25, 29) entsprechen, eingebracht wird und wenigstens ein weiteres pulverförmiges Material (28) in diejenigen Teile der Kapsel (40) eingebracht wird, die den Teilen der Brechschicht (20) entsprechen, welche den Vorsprung (24, 25, 29) umgeben, wobei das Material (27) des Vorsprungs (24, 25, 29), nachdem die Materialien (27, 28) isostatischem Heißpressen und anschließender Nachbehandlung unterworfen wurden, eine höhere Abrasionebeständigkeit besitzt als das Material (28) der Teile der Brechschicht (20), die den Vorsprung (24, 25, 29) umgeben.

20. Verfahren nach Anspruch 19, wobei der Vorsprung (24, 25, 29) in einem ersten Schritt durch isostatisches Heißpressen hergestellt wird, woraufhin die Teile der Brechschicht (20), die den Vorsprung (24, 25, 29) umgeben, in seinem zweiten Schritt hergestellt werden.

21. Verfahren nach einem der Ansprüche 14 bis 18, wobei die Brechschicht (20) wenigstens einen Vorsprung (24, 25, 29) aufweist, welcher von der Brechschicht (20) vorspringt und In einem ersten Schritt durch Sintern, Gießen oder Schmieden hergestellt wird, wobei der Vorsprung (24, 25, 29) in einem zweiten Schritt in der Kapsel (40) angeordnet wird und wenigstens ein pulverförmiges Material (28) in die Teile der Kapsel (40) eingebracht wird, die den Teilen der Brechschicht (20) entsprechen, welche den Vorsprung (24, 25, 29) umgeben, wobei der Vorsprung (24, 25, 29), nachdem die Materialien isostatischem Heißpressen und anschließender Nachbehandlung unterworfen wurden, eine höhere Abrasionsbeständigkeit besitzt als die Teile der Brechschicht (20), welche den Vorsprung (24, 25, 29) umgeben.

22. Verfahren nach einem der Ansprüche 19 bis 21, wobei der Vorsprung als eine Stufe (24, 25, 29) ausgebindet ist.

23. Verfahren nach einem der Ansprüche 14 bis 22, wobei der Hauptteil (19, 38) wenigstens teilweise aus einer Substanz hergestellt ist, die aus einer Gruppe ausgewählt ist, bestehend aus Kohlenstoffstählen und niedrig legierten Stählen.

## Revendications

1. Pièce d'usure pour concasseur rotatif ou concasser à mâchoires, adaptée pour être montée de manière détachable sur une partie support (10, 11) d'un concasseur (1) à action multiple, de type à impact, le concasseur (1) étant un concasseur rotatif ou un concasseur à mâchoires, **caractérisé en ce que** la pièce d'usure (5, 7, 34) est fabriquée au moins en partie par pressage isostatique à chaud, et **en ce que** la pièce d'usure (5, 7, 34) comprend un corps (19, 38) adapté pour monter la pièce d'usure (5, 7, 34) sur la partie support (10, 11) et une couche de concassage (20, 37, 39), attachée au corps (19, 38) et adaptée pour être mise en contact répété, durant le fonctionnement du concasseur (1), avec un matériau brut devant être concassé, le corps (19, 38) étant formé d'une substance aisée à usiner à des tolérances étroites, et la couche de concassage (20, 37, 39) étant formée d'un matériau (21, 22, 27, 28) présentant une haute résistance à l'abrasion.

2. Pièce d'usure selon la revendication 1, dans laquelle la couche de concassage (20, 37, 39) est formée d'au moins un matériau en poudre (21, 22, 27, 28) ayant été soumis à un pressage isostatique à chaud, et dans laquelle la substance dont est fait le corps (19, 38) présente également une bonne soudabilité.,

3. Pièce d'usure selon la revendication 1 ou 2, dans laquelle la couche de concassage (20, 37, 39) comprend au moins deux matériaux en poudre (21, 22, 27, 28), qui, sans être d'abord complètement mélangés les uns aux autres, ont été soumis à un pressage isostatique à chaud et lesdits matériaux (21, 22, 27, 28), après ledit pressage et un post-traitement subséquent, présentent des résistances à l'abrasion différentes, la couche de concassage (20, 37, 39), comprenant des parties (21', 22', 23, 24, 25, 26, 29) ayant des résistances à l'abrasion différentes.

4. Pièce d'usure selon la revendication 3, dans laquelle le matériau en poudre 22, 27) qui, après pressage et post-traitement subséquent, présente la résistance à l'abrasion maximale, est disposé dans les parties (22', 24, 25, 29) de la couche de concassage (20, 37, 39) où l'on s'attend à l'usure maximale.

5. Pièce d'usure selon l'une quelconque des revendications précédentes, dans laquelle la couche de concassage (20, 37, 39) et le corps (19, 38) sont joints par une zone de liaison (20').

6. Pièce d'usure selon l'une quelconque des revendications précédentes, dans laquelle le corps (19, 38) est formé au moins partiellement d'une substance sélectionnée parmi un groupe composé d'aciers au carbone et d'aciers faiblement alliés.

7. Pièce d'usure selon l'une quelconque des revendications précédentes, dans laquelle une première partie (21') de la couche de concassage (20) est formée d'au moins un premier matériau en poudre (21) et, en aval de ladite première partie (21') dans le sens d'écoulement (P) du matériau brut, une deuxième partie (22') de la couche de concassage (20) est formée d'au moins un deuxième matériau en poudre (22), qui, après que les matériaux (21, 22) aient été soumis à un pressage isostatique à chaud et à un post-traitement subséquent, présente une résistance à l'abrasion supérieure à celle du premier matériau (21), la deuxième partie (22') présentant une résistance à l'abrasion supérieure à celle de la première partie (21'),

8. Pièce d'usure selon la revendication 7, dans laquelle le premier matériau (21) fusionne graduellement en le deuxième matériau (22), d'une telle manière que la couche de concassage (20) reçoit une résistance à l'abrasion qui augmente graduellement en évoluant dans le sens de l'écoulement du matériau brut (P) et qui correspond à la charge d'usure en fonctionnement, de manière que le profil de la couche de concassage (20) soit conservé pratiquement intact pendant la durée de vie de la pièce d'usure (5, 7).

9. Pièce d'usure selon l'une quelconque des revendications 3, 4, 7 et 8, dans laquelle la couche de concassage (20) présente au moins une saillie (24, 25, 29) se projetant à partir de la couche de concassage (20) et composée d'au moins un matériau en poudre (27) qui, après avoir soumis les matériaux en poudre (27, 28) à un pressage isostatique à chaud et à un post-traitement subséquent, présente une résistance à l'abrasion supérieure à celle du matériau ou des matériaux en poudre (28) dont les parties de la couche de concassage (20) entourant la saillie (24, 25, 29) sont faites.

10. Pièce d'usure selon l'une quelconque des revendications 3, 4, 7 et 8, dans laquelle la couche de concassage (20) présente au moins une saillie (24, 25, 29) se projetant à partir de la couche de concassage (20) et réalisée par moulage, frittage ou forgeage et présentant une résistance à l'abrasion supérieure à celle du matériau ou des matériaux en poudre (28) dont les parties de la couche de concassage (20) entourant la saillie (24, 25, 29) sont faites.

11. Pièce d'usure selon l'une quelconque des revendications précédentes, constituent une enveloppe intérieure (5) ou une enveloppe extérieure (7), pour utilisation dans un concasseur rotatif (1).

12. Pièce d'usure selon la revendication 11 et l'une quelconque des revendications 9 et 10, dans laquelle la saillie présente la forme d'un gradin (24, 25, 29) répondant à une symétrie de rotation, s'étendant tout autour de la couche de concassage (20).

13. Pièce d'usure selon l'une quelconque des revendications précédentes, dans laquelle la couche de concassage (20) comprend au moins deux matériaux en poudre, qui, après avoir soumis les matériaux à un pressage isostatique à chaud, présentent des duretés différentes, le plus mou des deux matériaux étant situé dans une première couche (3 1) la plus proche du corps (19) et le plus dur des deux matériau étant situé dans une deuxième couche (32) située à l'extérieur de la première couche (31).

14. Procédé de fabrication d'une pièce d'usure, pour montage détachable sur une partie support (10, 11) dans un concasseur (1) à action multiple, de type à impact, le concasseur (1) étant un concasseur rotatif ou un concasseur à mâchoires,
**caractérisé en ce que** la pièce d'usure (5, 7, 34) est fabriquée sous forme de corps (19, 38), pour monter la pièce d'usure (5, 7, 34) sur la partie support (10, 11), et d'une couche de concassage (20, 37, 39), attachée au corps (19, 38) et adaptée pour être mise en contact répété, durant le fonctionnement du concasseur (1), avec un matériau brut devant être concassé, le corps (19, 38) étant formé d'une substance aisée à usiner à des tolérances étroites, et la couche de concassage (20, 37, 39) étant formée d'un matériau (21, 22, 27, 28) présentant une haute résistance à l'abrasion, par au moins un matériau en poudre (21, 22, 27, 28), introduit dans une capsule (40), la capsule (40) étant dégazée et fermée hermétiquement, et le matériau (21, 22, 27, 28) présent dans la capsule (40) étant soumis à un pressage isostatique à chaud, après quoi la pièce d'usure (5, 7, 34) est soumise à un post-traitement.

15. Procédé selon la revendication 14, dans lequel au moins deux matériaux en poudre (21, 22, 27, 28), qui, après avoir été soumis à un pressage isostatique à chaud et à un post-traitement subséquent, présentent des résistance à l'abrasion différentes, sont introduits dans la capsule (40) sans être complètement mélangés les uns aux autres, de telle manière que le matériau (22, 27) ayant la résistance à l'abrasion la plus haute soit disposé dans les parties de la capsule (40) correspondant aux parties (22', 24, 25, 29) de la couche de concassage (20, 37, 39) auxquelles l'on escompte une résistance à l'usure maximale.

16. Procédé selon la revendication 14 ou 15, dans lequel le corps (19, 38) de la pièce d'usure (5, 7, 34) est utilisé en tant que paroi dans la capsule (40) à joindre à la couche de concassage (20, 37, 39).

17. Procédé selon l'une quelconque des revendications 14 à 16, dans lequel au moins un premier matériau en poudre (21) est introduit dans une première partie de la capsule (40) qui correspond à une première partie (21') de la couche de concassage (20), et au moins un deuxième matériau en poudre (22) est introduit dans une deuxième partie de la capsule (40) qui correspond à une deuxième partie (22') de la couche de concassage (20), située en aval de la première partie (21') en observant dans le sens d'écoulement du matériau brut (P), le deuxième matériau (22), dans la deuxième partie (22"), après avoir soumis les matériaux (21, 22) à un pressage isostatique à chaud et à un post-traitement subséquent, ayant une résistance à l'abrasion supérieure à celle que présente le premier matériau (21).

18. Procédé selon la revendication 17, dans lequel le premier matériau (21) et le deuxième matériau (22) sont introduits dans la capsule (40), de manière que le premier matériau (21) fusionne graduellement en le deuxième matériau (22), la couche de concassage (20) recevant une résistance à l'abrasion allant en augmentant graduellement dans le sens d'écoulement du matériau brut (P) et correspondant à la charge d'usure en fonctionnement, de manière que le profil de la couche de concassage (20), soit maintenu pratiquement intact pendant la durée de vie de la pièce d'usure (5, 7).

19. Procédé selon l'une quelconque des revendications 14 à 18, dans lequel la couche de concassage (20), est fabriquée avec au moins une saillie (24, 25, 29) se projetant à partir de la couche de concassage (20), au moins un matériau en poudre (27) étant introduit dans la capsule (40), dans les parties de la capsule (40) correspondant à la saillie (24, 25, 29) et au moins un autre matériau en poudre (28) étant introduit dans les parties de la capsule (40) correspondant aux parties de la couche de concassage (20) entourant la saillie (24, 25, 29), le matériau (27) de la saillie (24, 25, 29), après avoir soumis les matériaux (27, 28) à un pressage isostatique à chaud et à un post-traitement subséquent, présentant une résistance à l'abrasion supérieure à celle du matériau (28) des parties de la couche de concassage (20) entourant la saillie (24, 25, 29).

20. Procédé selon la revendication 19, dans lequel la saillie (24, 25, 29) est fabriquée en une première étape, par un pressage isostatique à chaud, après quoi les parties de la couche de concassage (20) entourant la saillie (24, 25, 29) sont fabriquées, en une deuxième étape.

21. Procédé selon l'une quelconque des revendications 14 à 18, dans lequel la couche de concassage (20) présente au moins une saillie (24, 25, 29) se projetant à partir de la couche de concassage (20) et réalisée en une première étape, par frittage, moulage ou forgeage, la saillie (24, 25, 29), en une deuxième étape, étant agencée dans la capsule (40), et au moins un matériau en poudre (28) étant introduit dans les parties de la capsule (40) correspondant aux parties de la couche de concassage (20) entourant la saillie (24, 25, 29), la saillie (24, 25, 29), après avoir soumis les matériaux à un pressage isostatique à chaud et à un post-traitement subséquent, présentant une résistance à l'abrasion supérieure à celle de la couche de concassage (20) entourant la saillie (24, 25, 29).

22. Procédé selon l'une quelconque des revendications 19 à 21, dans lequel la saillie est formée sous forme d'un gradin (24, 25, 29).

23. Procédé selon l'une quelconque des revendications 14 à 22, dans lequel le corps (19, 38) est composé au moins partiellement d'une substance sélectionnée parmi un groupe composé d'aciers au carbone et d'aciers faiblement alliés.
